

Nov. 11, 1930.

C. K. STROBEL

1,781,088

RADIO DETECTOR

Filed Sept. 27, 1928



Fig. 1.



Fig. 2.



Fig. 3.



Fig. 4.



Fig. 5.



Fig. 6.

INVENTOR:  
C. K. Strobel,  
BY A. Z. Venecell  
His ATTORNEY

Patented Nov. 11, 1930

1,781,088

# UNITED STATES PATENT OFFICE

CHARLES K. STROBEL, OF PITTSBURGH, PENNSYLVANIA, ASSIGNOR TO THE UNION SWITCH & SIGNAL COMPANY, OF SWISSVALE, PENNSYLVANIA, A CORPORATION OF PENNSYLVANIA

## RADIODETECTOR

Application filed September 27, 1928. Serial No. 308,689.

My invention relates to radio detectors, and to methods of preparing the same.

I will describe two forms of radio detectors embodying my invention, and one method for preparing each of such forms, and will then point out the novel features thereof in claims.

In the accompanying drawing, Fig. 1 is a view showing, in side elevation, one form of radio detector prepared in accordance with my invention. Figs. 2, 3 and 4 are similar views showing another form of radio detector embodying my invention as it appears at different stages in the process of manufacture. Fig. 5 is a view showing, in side elevation, the detector illustrated in Figs. 2, 3 and 4, as it appears when completed. Fig. 6 is a view showing, in side elevation, the completed detector illustrated in Fig. 5 arranged for mounting.

Similar reference characters refer to similar parts in each of the views.

Referring first to Fig. 1, the reference character A designates in general a radio detector comprising a core, or bar B, of metal having a coating C of a compound of the metal formed thereon. For example, the bar B may be copper, and the compound of the metal may be cuprous oxide. The bar B may have any convenient size or shape, and the coating C may be formed thereon in any suitable manner. If the bar B consists of a bar of copper  $1'' \times \frac{1}{4}'' \times \frac{1}{16}''$ , a suitable coating of cuprous oxide may be formed thereon by heating the bar at a temperature of approximately  $1870^{\circ}$  F. for about twelve hours, and then allowing the bar to cool at atmospheric temperature. If a different size bar, or a different temperature is used, it may be necessary to heat the bar for a different length of time. After the bar has cooled, a portion of the oxide coating is broken away as indicated at E, to expose a portion of the bar. A fixed connection is then made to the exposed portion of the bar B by means of a wire 1. An adjustable connection is also made to the detector A by means of a fine wire 2, commonly known as a cat-whisker. The end of the wire 2 is brought into contact with the crystalline structure of the oxide coating at a

clean surface, such as the edge of the broken portion E. Or, if desired, a second portion of the oxide may be broken away as indicated at D, and the end of the wire 2 may be brought into contact with the crystalline structure of the oxide coating at the edge of this surface, as shown in the drawing.

I have found that a radio detector constructed in this manner possesses rectifying properties which are comparable with the rectifying properties of any of the heretofore known types of crystal detectors having asymmetric current characteristics, and this radio detector may be used in the same circuits as the heretofore known types of crystal detectors. Furthermore, a detector constructed in this manner is stable, and is comparatively easy to adjust.

In constructing the detector shown in Figs. 2, 3, 4 and 5, I employ a copper blank or bar F, having a tapered portion 3 at one end. This bar is heated in a furnace at a suitable temperature, such for example, as  $1870^{\circ}$  F., until the bar is completely oxidized, and the bar is then allowed to cool at atmospheric temperature. If a piece of #24 copper  $1\frac{1}{4}'' \times \frac{1}{4}''$  is used, the bar may be completely oxidized in about six hours. The bar then appears as shown in Fig. 3, and is designated by the reference character G. I next reduce the surface of the oxidized bar G to metallic copper in two portions, which are separated from each other by a narrow band of surface which is not reduced, and which preferably have a considerable difference in area. To accomplish this result, I cover the bar G near the small end of the tapered portion with a band H of some protecting material, such as paraffin, as shown in Fig. 4. I next immerse the bar G in a suitable electrolyte, such as dilute sulphuric acid, and pass a current through the electrolyte from a suitable anode to the bar as a cathode, thereby reducing the oxide to pure copper, until a coating or film of metallic copper having the desired thickness is obtained. The paraffin band is then removed by immersing the bar in hot water. The bar then appears as shown in Fig. 5, and has two portions J and K of its surface coated with a film of metallic copper, and a band L of its

surface which is not coated. Electrical connections are then made to the detector by a wire 5 soldered to the copper film of the portion K, and a wire 4 soldered to the copper film of the portion J.

It is sometimes desirable to arrange the detector in a manner convenient for mounting. For this purpose I have provided a glass tube M having two metallic end caps N and P (see Fig. 6). The detector is first placed in the tube M. One end cap N is then soldered to the wire 5, and the other end cap P is soldered to the wire 4. The end caps are then sealed on the glass tube in any convenient manner.

A detector constructed in this manner has good rectifying characteristics, and is mechanically rugged. The low resistance direction of such a detector is from the large area of reduced copper to the small area. I have found that different ratios of rectification may be obtained by varying the ratio of the small area of reduced copper to the large area.

I prefer to utilize a copper bar F having a tapered end 3, because this form of bar is convenient for obtaining a large difference in area between the two reduced portions J and K. This particular form of bar, however, is not essential to my invention.

Although I have herein shown and described only two forms of radio detectors embodying my invention, it is understood that various changes and modifications may be made therein within the scope of the appended claims without departing from the spirit and scope of my invention.

Having thus described my invention, what I claim is:

1. A radio detector comprising a bar of cuprous oxide having copper films formed on two separate portions of the bar having different areas.

2. A radio detector comprising a bar of cuprous oxide having copper films formed on two separate portions of a bar of cuprous oxide, the area of one said portion being several times the area of the other said portion.

3. A radio detector comprising a bar of cuprous oxide having a tapered end, and having a film of metallic copper on all but a small portion of the surface of the bar surrounding the bar near the small end of the tapered portion.

4. A radio detector comprising a bar of cuprous oxide having a tapered end and having a copper film on all but a small portion of its surface, said portion surrounding the bar at the tapered end in such manner that a comparatively small area of the copper film is separated from the remainder of the copper film.

5. In combination, a radio detector comprising a bar of cuprous oxide having a tapered end and having all of its surface

reduced to metallic copper with the exception of a small band surrounding the bar near the end of the tapered portion, a protecting tube surrounding said bar, electrically conducting end caps sealed on said tube, and means for connecting the copper film of the bar at the opposite ends of the bar with the adjacent end cap.

In testimony whereof I affix my signature.

CHARLES K. STROBEL.

75

80

85

90

95

100

105

110

115

120

125

130